

Nov. 16, 1937.

C. S. HAMERSLEY ET AL

2,099,301

PAPER WRAPPER FOR COMMODITIES

Filed Sept. 21, 1933

Fig. 1



Fig. 2



Fig. 3



Fig. 4



Fig. 6



Fig. 5



## UNITED STATES PATENT OFFICE

2,099,301

## PAPER WRAPPER FOR COMMODITIES

Carl S. Hamersley, New York, N. Y., and Sumner C. Fairbanks, Passaic, N. J.; said Fairbanks assignor to said Hamersley

Application September 21, 1933, Serial No. 690,394

10 Claims. (Cl. 229—87)

Our present invention relates generally to the wrapping art, and has particular reference to a new and improved wrapper of sheet material such as paper.

5 While we have herein illustrated, and shall hereinafter describe, a transparent paper wrapper of the character which is designed primarily for use in wrapping a commodity such as a bread loaf, nevertheless it will be understood that certain phases of our invention are not necessarily restricted to this particular type of wrapper or to this particular use.

10 A general object of our invention is to provide an improved wrapper whose application around a commodity is facilitated and rendered more secure. More particularly, we aim to provide an improved paper wrapper having opposite margins which are adapted to be folded and sealed, under heat and pressure, when the wrapper is applied to the article. In accordance with our present invention, these opposite margins are coated with a bonding material of unique and novel characteristics, whereby the efficiency of the sealing procedure is increased.

15 It is a more particular object to provide an improved wrapper of the waxed paper type, although certain phases of our invention are not necessarily restricted to sheet material of this character.

20 In the wrapping of bread, cake, and similar commodities, it is customary practice to employ a wrapper of waxed paper or the equivalent, and to effect the actual wrapping procedure by means of a machine which tucks in the opposite ends of the wrapper, folds them, and applies heat and pressure for the purpose of melting the wax and thereby effecting a wax bond between the interleaved ends of the wrapper. The sealing effect which is thus produced is quite satisfactory, but from a number of aspects it is not adequately secure; and by means of our present invention we have provided a wrapper which is adapted to be sealed around such a commodity with greater security and firmness.

25 The problems involved in providing a wrapper of improved sealing qualities are peculiar. The mere use of a conventional type of adhesive is unfeasible. If the adhesive is to be applied in a moist condition at the wrapping machine, it impairs the smooth operation of the latter, and it is a messy proceeding which is thoroughly undesirable, especially since edible commodities are being handled by the wrapping machine at the same time. If the adhesive is applied to the wrapper during its manufacture, so that it is merely necessary to wet the adhesive with water or similar

solvent at the time of the wrapping, the same objections obtain.

Apart from the foregoing reasons which prevent an ordinary adhesive to be used, an added difficulty presents itself when the wrapper is of waxed paper, because the adhesive must be of a character which will not only adhere to the wax but which will penetrate through the wax when the sealing is to be effected; and ordinary adhesives do not meet with these requirements.

30 It is a feature of our present invention to provide a bonding material which is readily applicable to the wax during the initial manufacture of the wrapper; which is normally of no appreciable viscosity; and which is adapted to become operative under the mere application of heat and pressure, requiring no messy procedure at the wrapping machine and permitting the latter to function in its normal manner. The bonding material of our present invention has the characteristic of becoming substantially tacky under the slight temperature rise which is produced at the wrapping machine; and it has the special advantage of being adapted to penetrate through the wax and to effect a firm bonding action with the paper itself when heat and pressure are applied.

35 It is another feature of our invention to provide a wrapper in which certain opposite margins are coated with a bonding material of the foregoing type, and in which the midportion of the wrapper, between said margins, is purposely thickened to a degree which makes the midportion at least as thick as the coated margins. This permits the wrapper to be formed as a continuous roll, which may be cut into suitable wrapper blanks at the wrapping machine. If the midportion were not thickened, the thickness at the margins would prevent the material from being efficiently wound into rolled form.

40 Our invention is predicated upon the discovery that resins, in general, and certain specific resins (preferably synthetic), in particular, embody the desirable characteristics which are necessary to accomplish the present objectives. The bonding material which we employ is, therefore, composed essentially of a resin, mixed with just sufficient plasticizer to destroy the natural brittleness of the resin, and to lower the melting point to approximately the melting temperature of wax. A 45 mixture of this character is unreactive toward wax; has no appreciable normal viscosity; becomes substantially tacky when subjected to a slight temperature rise; and has the important advantage of penetrating through the wax to 50

55

form a secure bond with the paper itself when heat and pressure are applied. The latter ability of the present material is probably due to the fact that its viscosity is greater than that of wax.

5 We achieve the foregoing objects and advantages, and such other objects and advantages as may hereinafter appear or be pointed out, in the manner illustratively exemplified in the accompanying drawing, wherein—

10 Figure 1 is a diagrammatic view of the manner in which a strip of wrapping material of the present character may be advantageously manufactured;

15 Figure 2 is an enlarged cross-sectional view taken substantially along the line 2—2 of Figure 1;

20 Figure 3 is a plan view of a section of the completed strip of wrapping material of the type produced by the apparatus of Figure 1;

25 Figure 4 is an enlarged cross-sectional view taken substantially along the line 4—4 of Figure 3;

30 Figure 5 is a perspective view of a wrapped bread loaf or the like; and

35 Figure 6 is an enlarged fragmentary cross-section through certain interleaved and sealed layers of the material, showing the manner in which the sealing is accomplished.

40 In accordance with one method of carrying out our present invention, a main roll of suitable paper 10 is caused to be guided around a guide roller 11 submerged in a bath of molten wax 12. At the same time, an auxiliary roll 13 of narrower material is similarly caused to be guided around 45 a guide roller 14 submerged in the bath 12, whereby the two wax-coated strips may then be caused to pass simultaneously between a pair of pressure rollers 15 as they emerge from the bath. The strip 13 is arranged in a manner whereby it will overlie the longitudinal midportion of the main sheet 10, and the step of passing between the rollers 15 results in squeezing out excess wax and at the same time firmly bonding the narrower strip 13 to the main strip 10.

45 This assembly is then caused to pass over two or more doctor rolls 16 which dip into a bath or baths 17 of the present type of bonding material. Preferably, each of the rolls 16 is formed of a series of spaced discs, as shown most clearly in 50 Figure 2, whereby the bonding material 17 is applied to the marginal portions of the sheet 10 along a series of substantially parallel line areas. This produces a series of ridges 18 of the bonding material, as shown most clearly in Figure 4.

55 The resultant strip is then passed over suitable cooling rollers, and is ultimately wound onto a mandrel or drum. A section of the resultant strip is shown most clearly in Figures 3 and 4. It will be observed that the medial band 13 is 60 securely bonded to the main strip 10 by means of an intermediate layer of wax 19, and that the entire sheet is surrounded and enveloped by a similar layer of homogeneous wax. This coating is designated by the reference numeral 20 in

65 Figure 4. The medial strip or band 13 may serve a dual function. In the first place, it thickens the midportion of the wrapping material between the coated margins, so that the resultant thickness at the midportion is greater than that of the body portion of the material, and is at least as thick as the coated margins. This permits the material to be rolled efficiently onto a drum or the like, since the midportion of the roll is thereby permitted to form a solid mass which is firmly 70 compacted and which holds the roll in a stable

condition. The edge portions of the roll are relatively uncompacted, being thinner, but this does not interfere with the stability of the roll as would be the case if the edge portions were thicker than the midportion. The other purpose 5 which the band 13 may fulfill is to embody on its inner face a layer of printed indicia 21 which is thus caused to show through the sheet 10 in a remarkably efficient and attractive manner, making it appear as though the printing or 10 similar legend were actually on the outer face of the wrapper. By "outer face" we refer to the surface which is uppermost in Figure 4, and it is this surface which is exposed outwardly when the wrapper is applied to a commodity. 15

Obviously, the medial band 13, which may be of paper or similar material, serves also to reinforce the wrapper at the midportion thereof; and when an individual wrapper blank is enveloped around a commodity, such as a bread loaf, as 20 shown in Figure 5, the medial band 13 serves as an efficient reinforcement for the entire wrapped commodity.

The bonding material which we employ is unreactive toward wax, and is adapted to be efficiently applied to the wax, as shown at 18 in Figure 4, this application being preferably accomplished in the manner shown in Figures 1 and 2. Under normal conditions, the ridges or masses of bonding material 18 are of no appreciable viscosity and rest substantially on the outer surface of the wax coating 20, although perhaps a slight merging of the ridges with this layer of wax may take place. This normally dry condition of the wrapper permits it to be efficiently 35 rolled, packed, shipped, and handled, without any special precautions, and without any likelihood of annoying tackiness. When the wrapper is used, however, the advantageous characteristics 40 of our present bonding material become manifest.

We have not illustrated a wrapping machine, nor is our invention restricted to the use of any particular type of wrapping machine, but it will be understood that severed blanks of the wrapping material are caused to be enveloped around a commodity so that the ends may be interfolded in the manner designated generally by the reference numeral 22 of Figure 5. Heat and pressure are then applied to these ends, and when 50 this is done the wax and the bonding material melt. The bonding material being of greater viscosity than the wax, each mass of the material penetrates through the wax beneath it and comes into direct contact with the paper. Under 55 pressure, a direct and highly efficient and tenacious bond is thus effected between the two layers of superposed paper; and as soon as the wrapping machine discharges the product, the wax and the bonding material resume their normal 60 untacky condition and become hard and non-viscid.

The efficiency with which the bond is effected is shown most clearly in Figure 6, in which 23 and 24 designate two superposed layers of the paper, the sheet 23 being coated on opposite sides with the wax layers 25 and 26; and the sheet 24 being coated on opposite sides with the wax layers 27 and 28. The line 29 is shown in dot-and-dash, because it exists before the heat and 70 pressure are applied but disappears when the layers 26 and 27 melt and merge with each other. The two masses 30 of the present bonding material are illustrative of the manner in which the areas or ridges 18 are believed to act under the 75.

heat and pressure that is applied. The material may originally have rested on the layer 26, or on the layer 27, or both, but in any event the melting of the material causes it to penetrate through the wax layers 26 and 27 until it comes into direct contact with the superposed paper layers 23 and 24. This action is no doubt due to the relatively greater viscosity which the bonding material has. When the heat and pressure treatment is completed, and the wrapped commodity is discharged by the wrapping machine, the bond effected, as shown in Figure 6, remains as an efficient bond which is far more tenacious than that effected by the mere merging of the wax layers 26 and 27.

It will be understood that at the folded and sealed ends of the wrapped commodity there will sometimes be more than two layers of paper bonded together in the manner shown in Figure 6, and Figure 6 cannot be said to be the cross-section along a specific line of Figure 5 for this reason. However, the action illustratively shown in Figure 6 as taking place between two superposed layers of paper takes place in substantially the same manner wherever masses of the bonding material 18 encounter an adjacent layer of the material under heat and pressure.

While we have found that resins, in general, may be employed for our present purpose, we prefer to use a resin of the class which includes coumarone-indene, ester gum, gum dammar, kauri gum, copal, and the like. Of these, we have found coumarone-indene to be particularly advantageous and useful in carrying out our present objectives. Whatever resin is used will be mixed with a sufficient amount of plasticizer to lower the melting point of the mixture to substantially that of wax. While any well known type of plasticizer may be employed, depending largely upon choice, we prefer to use a plasticizer of the class which includes tri-cresyl-phosphate, di-butyl-phthalate, tri-phenyl-phosphate, chlorinated diphenyl, and the like. Of these, we prefer tri-cresyl-phosphate, and, in fact, a satisfactory bonding material may consist, for example, of a mixture of about 72% of coumarone-indene and about 28% of tri-cresyl-phosphate.

Modifications in the proportions may obviously be made by those skilled in the art to meet differing requirements of melting temperature and the like. Care should be taken, however, to add just enough plasticizer and not too much, because if an excess amount of plasticizer is used the mixture may partake of an undesirable viscosity under normal conditions. Similarly, if insufficient plasticizer is used, the bonding material may not melt to a sufficient degree when the heat and pressure of the wrapping machine are applied.

While we have illustrated and described our invention in connection with a continuous strip of wrapping material, it will be understood that this is merely a preferred method of carrying out our general objectives, and that our invention is not necessarily restricted to any continuous method of manufacture or use. Similarly, while we have shown the manner in which our invention may be employed in connection with waxed paper, since this is the preferred type of paper in many instances, nevertheless many phases of our invention, including the bonding material and its method of use, are not restricted to employment with waxed paper. Ordinary glassine paper or regenerated cellulose may be similarly coated along its margins with the present type

of bonding material, and may be thickened at the midportion in the manner hereinbefore described to carry out the general purposes of our invention.

Furthermore, while we have illustratively shown the preferred manner of thickening the midportion of the wrapper by means of an extra strip or band of paper or the like, nevertheless it will be understood that this thickening may be accomplished in other ways, as, for example, by interleaving a separate strip of material with the wrapping material without necessarily bonding it thereto by means of wax; also by thickening the midportion by the addition of extra wax; or in other ways which will suggest themselves to those skilled in the art.

Wherever we have used the term "normal" herein and in the appended claims, we refer to room temperature conditions. By the same token, the term "slight temperature rise" refers to an increase of temperature of the type which is accomplished by heat at a wrapping machine; and we do not mean to allude either to temperature rises of lesser degree nor to extreme temperature rises that are not encountered in ordinary use of wrappers of the present character.

The term "wax" includes, of course, such materials as paraffin or the like which are customarily used in the manufacture of what is usually referred to as waxed paper.

In general, it will be understood that changes in the details, herein described and illustrated for the purpose of explaining the nature of our invention, may be made by those skilled in the art without departing from the spirit and scope of the invention as expressed in the appended claims. It is, therefore, intended that these details be interpreted as illustrative, and not in a limiting sense.

Having thus described our invention, and illustrated its use, what we claim as new and desire to secure by Letters Patent is—

1. A waxed paper wrapper having along certain margins a coating of bonding material which is unreactive toward wax and of no appreciable normal viscosity, said material having a greater viscosity than wax and being substantially tacky at the melting temperature of wax.

2. A waxed paper wrapper having along certain margins a coating of bonding material which is unreactive toward wax and of no appreciable normal viscosity, said material having a greater viscosity than wax and being substantially tacky at the melting temperature of wax; said material consisting essentially of a resin.

3. A waxed paper wrapper having along certain margins a coating of bonding material which is unreactive toward wax and of no appreciable normal viscosity, said material having a greater viscosity than wax and being substantially tacky at the melting temperature of wax; said material consisting essentially of a resin of the class which includes coumarone indene, ester gum, gum dammar, kauri gum, and copal.

4. A waxed paper wrapper having along certain margins a coating of bonding material which is unreactive toward wax and of no appreciable normal viscosity, said material having a greater viscosity than wax and being substantially tacky at the melting temperature of wax; said material consisting essentially of coumarone indene.

5. A waxed paper wrapper having along certain margins a coating of bonding material which is unreactive toward wax and of no appreciable normal viscosity, said material having a greater

viscosity than wax and being substantially tacky at the melting temperature of wax; said material comprising a resin mixed with a plasticizer.

6. A waxed paper wrapper having along certain margins a coating of bonding material which is unreactive toward wax and of no appreciable normal viscosity, said material having a greater viscosity than wax and being substantially tacky at the melting temperature of wax; said material 10 consisting of a resin mixed with just sufficient plasticizer to lower the melting point of the mixture to substantially that of wax.

7. A waxed paper wrapper having along certain margins a coating of bonding material which 15 is unreactive toward wax and of no appreciable normal viscosity, said material having a greater viscosity than wax and being substantially tacky at the melting temperature of wax; said material comprising a resin mixed with a plasticizer of the 20 class which includes tri-cresyl-phosphate, di-butyl-phthalate, tri-phenyl-phosphate, and chlorinated diphenyl.

8. A waxed paper wrapper having along certain margins a coating of bonding material which

is unreactive toward wax and of no appreciable normal viscosity, said material having a greater viscosity than wax and being substantially tacky at the melting temperature of wax; said material comprising a mixture of coumarone indene and a 5 plasticizer.

9. A waxed paper wrapper having along certain margins a coating of bonding material which is unreactive toward wax and of no appreciable normal viscosity, said material having a greater 10 viscosity than wax and being substantially tacky at the melting temperature of wax; said material comprising a mixture of coumarone indene and tri-cresyl-phosphate.

10. A waxed paper wrapper having along certain margins a coating of bonding material which is unreactive toward wax and of no appreciable normal viscosity, said material having a greater viscosity than wax and being substantially tacky at the melting temperature of wax; said material 20 consisting of a mixture of about 72% coumarone indene and about 28% tri-cresyl-phosphate.

CARL S. HAMERSLEY.  
SUMNER C. FAIRBANKS.